

# United States Patent [19]

Brunko

[11] 3,779,817

[45] Dec. 18, 1973

[54] **METHOD OF PRODUCING QUENCHED AND TEMPERED HOLLOW STEEL STRUCTURAL MEMBERS OF POLYGONAL CROSS SECTION**

[75] Inventor: **Wade D. Brunko**, Library, Pa.

[73] Assignee: **United States Steel Corporation**, Pittsburgh, Pa.

[22] Filed: **Sept. 25, 1972**

[21] Appl. No.: **291,854**

[52] U.S. Cl. .... **148/12.4**

[51] Int. Cl. .... **C21d 9/08**

[58] Field of Search ..... 148/12.4

[56] **References Cited**

UNITED STATES PATENTS

2,222,263 11/1940 Nelson ..... 148/12.4

2,256,455 9/1941 Crawford ..... 148/12.4  
2,748,039 5/1956 Adams et al. .... 148/12.4

Primary Examiner—W. W. Stallard

Attorney—Ralph H. Dougherty

[57]

## ABSTRACT

Method of producing quenched and tempered hollow steel structural members of polygonal cross section includes the steps of hot rolling a hollow steel tube, austenitizing the tube, water quenching it, reheating the tube to a tempering temperature just below the lower critical transformation temperature, and rolling the tube to the desired polygonal cross section while holding the temperature of the member at the tempering temperature.

8 Claims, No Drawings

**METHOD OF PRODUCING QUENCHED AND TEMPERED HOLLOW STEEL STRUCTURAL MEMBERS OF POLYGONAL CROSS SECTION**

This invention relates to hollow steel structural tubing, and more particularly to quenched and tempered structural steel tubing of polygonal cross section such as square or rectangular. Tubular structural steels processed in this manner developed high yield strengths and high tensile strengths, together with high notch toughness at low temperatures.

Heretofore, structural steel tubing of polygonal cross sections has been produced in one of two ways. In the first method, a substantially round tube is formed by hot rolling in a tube mill, which tube is formed into the desired cross sectional dimensions and shape by passing it through a squaring pass after the round tube has been formed. The squaring or sizing operation is carried out at a temperature of from about 1100° to 1500°F. In the second method, the tube is hot rolled in a conventional manner, then reheated to about 1300°F., and passed through a sizing mill to form the tube into a polygonal cross section. Heat treatment of the finished shapes has resulted in distortion of the flat faces of the shapes beyond acceptable commercial limits. Thus, the physical properties such as strength and toughness of these tubes are limited to those properties which can be attributed to chemical composition alone. US Pat. No. 2,748,039 teaches a method of producing a quenched and tempered pipe of round cross section which requires additional small reductions to be made after the quench and temper process to remove minor distortions caused thereby.

This invention is predicated upon my development of a weldable water-quenched and tempered structural tube of polygonal cross section to meet the demand for higher strength structural materials with superior notch toughness properties.

Accordingly, it is the principal object of this invention to provide a method of producing quenched and tempered hollow steel structural members of polygonal cross section having high yield strengths, and excellent notch toughness and elongation properties.

It is a further object of this invention to provide a method of producing dimensionally correct hollow steel structural members.

The method of the invention consists of:

- a. Hot rolling a hollow steel tube with substantially oval or circular cross section by any conventional tube rolling method;
- b. Austenitizing the tube;
- c. Water quenching the tube to about 150°F;
- d. Reheating the tube to a temperature above the stress relieving temperature and below the  $Ac_1$  temperature;
- e. Tempering the tube in the tempering temperature range;
- f. Rolling the tube to the desired polygonal cross section while holding the temperature of the tube

within the tempering temperature range; and

g. Allowing the resulting product to be air cooled.

The chemical composition of the steel in the tube may be any steel which is suitable for the production of quenched and tempered tubes. A suitable composition is a silicon-aluminum killed steel, having a composition of about 0.20% carbon, 1.45% manganese and 0.06% vanadium. This steel composition is martensitic and exhibits good weldability.

10 Austenitizing is accomplished at a temperature greater than the  $A_3$  temperature of the steel in the tube. For most steels, this means a temperature greater than 1550°F but will usually be from about 1600°F to about 1750°F. Preferably, the austenitization is carried out in 15 a gas-fired furnace in an excess air atmosphere for a sufficient time to assure uniform heating of the tube.

Water quenching is accomplished by passing the tube through a series of spray quench rings to provide 100% surface coverage of the tube circumference. The tube 20 is quenched to a temperature of about 150°F, but may be quenched to any temperature below 200°F.

The tempering temperature is just above the stress 25 relieving temperature and just below the lower critical transformation temperature of the steel, that is, just below the  $Ac_1$  temperature. For most steels, tempering will be carried out at a temperature between about 1150°F and 1225°F. The tube is tempered for a period sufficient to bring the tube to a uniform tempering temperature.

30 The tube is rolled to the desired polygonal cross section such as a round-cornered square, round-cornered rectangle or any other desired cross section while within the tempering temperature range. This is normally done with a sizing mill having a number of stands 35 with squaring passes.

The shapes produced by this method are free of distortion, have high notch toughness, high yield strength and high ultimate strength.

To illustrate the present invention, two steels having 40 chemical compositions as shown in Table 1 were melted in an electric furnace and rolled into 10 inch diameter tube rounds which were subsequently rolled into 10  $\frac{1}{8}$  inch outside diameter seamless tubes, half of each composition having three-eighths inch walls and 45 half having one-half inch walls. The lower vanadium content tubes were austenitized at 1600°F, and the higher vanadium tubes at 1650°F, in a walking beam furnace for 100 minutes per inch of wall thickness. This was followed by spray quenching with quench water at a temperature of about 92°F. The one-half inch wall tubes were quenched at a speed of 26 ft. per minute and the three-eighths inch wall tubes at 36 ft. per minute. The tubes were regrouped and some were tempered at 1175°F, and some at 1225°F. All tempering was for 72 minutes total furnace time, after which the round tubes were formed into square tubes at the tempering temperature in a five-stand sizing mill having squaring passes. The final tubes were allowed to air cool.

TABLE I

|                  | C   | Mn   | P     | S     | Si   | Al    | V     | Cu   | Ni   | Cr   | Mo   | N <sub>2</sub> |
|------------------|-----|------|-------|-------|------|-------|-------|------|------|------|------|----------------|
| Ingot No. 1..... | .22 | 1.49 | 0.011 | 0.019 | 0.45 | 0.064 | 0.037 | 0.01 | 0.16 | 0.08 | 0.01 | 0.008          |
| Ingot No. 2..... | .22 | 1.51 | .009  | .019  | .47  | .067  | .071  | .01  | .16  | .08  | .01  | .....          |

Table 2 shows the mechanical properties from two as-rolled tensile tests and tests from each tube quenched and tempered according to this process. From this data, it is clear that 75,000 psi minimum yield strength may be attained in all wall thicknesses to 5

above the stress relieving temperature and below the  $A_c$  temperature;  
e. tempering said tube at said tempering temperature;  
f. rolling said tube to the desired polygonal cross-section while within said tempering temperature range; and

TABLE 2

| Pipe No. and end | Composition | Wall   | Austenitizing temperature | Temper temperature (°F.) | Longitudinal strip tensile |                         |                  |               |
|------------------|-------------|--------|---------------------------|--------------------------|----------------------------|-------------------------|------------------|---------------|
|                  |             |        |                           |                          | Yield strength (psi)       | Ultimate strength (psi) | Elong. in 2" (%) | Yield tensile |
| 1E-S.....        | 0.04 V..... | 0.500" | As-rolled.....            | 68,490                   | 98,480                     | 32.0                    | 0.70             |               |
| 2E-S.....        | 0.07 V..... |        |                           | 74,070                   | 103,790                    | 28.5                    | .72              |               |
| 1A-N.....        | 0.04 V..... | .375"  | 1600 °F.....              | 1175                     | 88,630                     | 102,980                 | 30.0             | .86           |
| 1B-S.....        |             |        |                           | 1175                     | 89,770                     | 103,300                 | 27.5             | .87           |
| 1C-N.....        |             |        |                           | 1225                     | 79,400                     | 94,350                  | 34.0             | .84           |
| 1D-S.....        |             |        |                           | 1225                     | 80,300                     | 95,460                  | 35.0             | .84           |
| 1E-N.....        |             | .500"  |                           | 1175                     | 86,090                     | 100,680                 | 33.0             | .86           |
| 1G-S.....        |             |        |                           | 1225                     | 82,590                     | 94,200                  | 35.0             | .88           |
| 1I-N.....        |             |        |                           | 1225                     | 80,800                     | 95,220                  | 35.0             | .85           |
| 2A-N.....        | 0.07 V..... | .375"  | 1650 °F.....              | 1175                     | 98,070                     | 111,420                 | 30.0             | .88           |
| 2B-S.....        |             |        |                           | 1175                     | 102,990                    | 114,480                 | 29.0             | .90           |
| 2C-N.....        |             |        |                           | 1225                     | 91,420                     | 104,790                 | 31.0             | .87           |
| 2D-S.....        |             |        |                           | 1225                     | 95,440                     | 100,260                 | 32.5             | .95           |
| 2E-S.....        |             | .500"  |                           | 1175                     | 90,670                     | 106,680                 | 31.0             | .85           |
| 2G-N.....        |             |        |                           | 1225                     | 84,590                     | 101,200                 | 33.5             | .84           |
| 2I-S.....        |             |        |                           | 1225                     | 85,360                     | 102,610                 | 36.0             | .83           |

Charpy V-notch impact properties were excellent with 100% shear and 93 ft./lbs. of energy absorption on a two-thirds size specimen at minus 100°F.

From the foregoing, it can readily be seen that I have invented a method of producing dimensionally correct quenched and tempered hollow steel structural members of polygonal cross section having high yield strength, excellent notch toughness and excellent elongation properties.

I claim:

1. A method of producing hollow steel structural members of polygonal cross-section comprising:
  - a. hot-rolling a hollow steel tube of substantially round cross-section;
  - b. austenitizing said tube at a temperature greater than the  $A_3$  temperature of the steel in said tube;
  - c. water quenching said tube;
  - d. reheating said tube to a tempering temperature

45

g. air cooling said tube.

2. A method according to claim 1 wherein said austenitizing temperature is above 1550°F.

3. A method according to claim 2 wherein said austenitizing temperature is from about 1600°F to about 1750°F.

4. A method according to claim 1 wherein said tube is water quenched to a temperature below about 200°F.

5. A method according to claim 4 wherein said tube is water quenched to a temperature of about 150°F.

6. A method according to claim 1 wherein said tempering temperature is from about 1150°F to about 1225°F.

7. A method according to claim 1 wherein said polygonal cross-section is a round-cornered rectangle.

8. A method according to claim 1 wherein said polygonal cross-section is a round-cornered square.

\* \* \* \* \*

50

55

60

65